# EUROPEAN PATENT SPECIFICATION

(11) **EP 0 833 783 B1**
(45) Date of publication and mention of the grant of the patent: **16.08.2000**
(21) Application number: 96919353.1
(22) Date of filing: 06.06.1996
(51) Int. Cl.: B65D 51/24, B65D 53/00, B65D 53/04, B65D 53/06, B05D 7/22

(54) **AN OXYGEN ABSORBING CONTAINER CAP LINER**
SAUERSTOFFABSORBIERENDE AUSKLEIDUNG EINER BEHÄLTERKAPPE
REVETEMENT INTERNE DE BOUCHON DE RECIPIENT ABSORBANT L'OXYGENE

(30) Priority: 06.06.1995 US 471573
(43) Date of publication of application: 08.04.1998
(73) Proprietor: Multisorb Technologies, Inc., Buffalo, NY 14224-1893 (US)
(72) Inventor: McKDEY, George, E., Williamsville, NY 14221 (US)
(74) Representative: Sandmair, Kurt, Dr. Dr.
(86) International application number: US9610036
(87) International publication number: WO9639338

(56) References cited:
- WO-A-91/17044
- US-A- 3 695 477
- US-A- 3 866 845
- US-A- 4 287 995
- US-A- 4 785 952
- US-A- 5 381 914

## Description

### FIELD OF THE INVENTION

This invention relates in general to oxygen absorbents. It relates in particular to an oxygen absorbent dispersed in a liner of a container cap.

### BACKGROUND OF THE INVENTION

Many products are susceptible to putrefaction, denaturation, mold growth, spoilage, rancidity, oxidation, or other deterioration when brought into contact with oxygen. Examples of such products include beer, wine, juice, vinegar, sauces, seasonings, processed foods, bread, produce, meats, and certain pharmaceuticals and chemicals, among a variety of others. Preservation of such products is disturbed when molds, bacteria, and other organisms that thrive in the presence of oxygen are present. These organisms cause the putrefaction and change in the taste or quality of the product. In addition, some of the products themselves are liable to be affected by oxidation that changes the taste or quality of the product. To prevent such oxidation and growth of organisms and thus increase the preservation stability of these products, the oxygen must be removed from the container in which the products are stored.

One technique for avoiding or reducing the presence of oxygen is vacuum packing. This involves evacuating a container before charging it with the product. Another technique is gas displacement. Here, an inert gas such as nitrogen is used to displace the air and hence the oxygen in a container. The displacement can be performed before or after the product is charged to the container.

Still another technique is a foaming method. Particularly applicable to products such as beer, a jet foamer can be used to inject a small amount of pressurized water to foam the beer after charging it to the container. The foam acts as a mechanical deoxygenizer, forcing the oxygen from the container.

Common disadvantages associated with all of the above techniques are the requirement of large-scale apparatus and operation and the difficulty of removing oxygen dissolved in the product. Also, in general, these techniques leave between 0.2% and 5.0% of the oxygen in the container. This amount of oxygen in the container is enough to adversely affect most products.

A simpler, more efficient technique for oxygen removal involves placing an oxygen absorbent in the container with the product. For this purpose, it is known to attach an oxygen absorbent to the underside of a container cap. For example, in U.S. Patent No. 4,287,995, issued to Moriya, an oxygen absorbent is placed on the underside of a cap. The oxygen absorbent is held in place by a cover layer of gas permeable film that prevents contact between the absorbent and the contents of the container.

U.S. Patent No. 5,143,763, issued to Yamada et al., discloses a multi-layer composition adapted to be attached to a liner on the underside of a container cap. The layers of the composition include (1) an adhesive layer that attaches the multi-layer structure to the cap liner, (2) an oxygen absorbing layer consisting of an oxygen absorbent dispersed in a resin, and (3) an oxygen permeable film layer covering the absorbent layer. The oxygen permeable film layer prevents the oxygen absorbent from leaching out from the resin into the contents of the container. The adhesive layer is disposed between the cap liner and the oxygen absorbing layer, completely separating the cap liner.from the oxygen absorbing layer. A similar lines comprising several layers is disclosed in US-A- 5 381 914.

U.S. Patent No. 5,274,024, issued to Koyama et al., also discloses a multi-layer composition adapted to be attached to the underside of a container cap. The patent discloses an adhesive layer, used to attach an oxygen absorbent layer to the cap, and an outer layer over the oxygen absorbing layer. The outer layer prevents direct contact between container contents and the oxygen absorbent. Again, the adhesive layer is disposed between the cap and the oxygen absorbent layer, completely separating the cap from the oxygen absorbent layer.

Another container closure is disclosed in WO 91/17 044.

In all of the known devices, however, separate layers are used to accomplish the functions of lining the container cap, adhering the oxygen absorbent to the cap, absorbing the oxygen, and covering the oxygen absorber to prevent it from contacting the contents within the container.

### SUMMARY OF THE INVENTION

The present invention provides a container cap according to claim 1. Preferred embodiment are as set forth in claim 2.

The present invention also provides a method according to claim 3. Preferred embodiments are as set forth in claims 4 and 5.

### BRIEF DESCRIPTION OF THE DRAWING

Fig. 1 is a cross-sectional side view of an oxygen absorbing container cap in accordance with an exemplary embodiment of the present invention;
Fig. 2 is a perspective view in partial cross-section of an oxygen absorbing container cap in accordance with an exemplary embodiment of the present invention;
Fig. 3 is a partially cross-sectional side view of an oxygen absorbing container cap attached to a container in accordance with an exemplary embodiment of the present invention;
Fig. 4 is a cross-sectional side view of an oxygen absorbing cap in accordance with another exemplary embodiment of the present invention; and
Fig. 5 is a top view of the embodiment shown in Fig. 4.

### DETAILED DESCRIPTION OF THE INVENTION

The present invention provides an oxygen absorbing cap according to claim 1 with an oxygen absorbent dispersed in a liner of the cap, the liner being directly attached to the inside surface of the cap. No cover layer is used over the liner. When such a cap is secured to a container, the oxygen absorbing liner in the cap acts both as a sealant, providing a seal between the cap and the container, and as an oxygen absorber, removing oxygen from inside the container. A similar liner is known disclosed in WO 91/17 044. The document, however, discloses organic compounds or metal chelates as the oxygen scavanges.

Fig. 1 shows a side view of an exemplary embodiment of the present invention. Cap 11 includes a base portion 20 and a cylindrical portion 21 that is typically integrally formed with base portion 20. Cap 11 may be a plastic material, such as polyvinylchloride, polystyrene, or polycarbonate. Cap 11 may also be a metallic material, such as aluminum or iron. Grooves 13 are formed on the inner surface of cap 11 to mate with threads on a container opening (not shown).

Liner 12 is disposed on the inner surface of cap 11. Liner 12 in the illustrated embodiment includes a carrier resin with an oxygen absorbing material dispersed therein.

The oxygen absorbing materials useful in the present invention include 200 mesh iron, solid electrolytic salts, and glucose oxidase. The 200 mesh iron may be hydrogen-reduced iron, electrolytically reduced iron, or chemically reduced iron. Although iron is preferred as the metallic oxygen absorbing agent, it will be appreciated that other metals may be used. These are, by way of example and not limitation, aluminum, copper, zinc, titanium, magnesium, and tin. These other materials do not, however, absorb oxygen as fast as iron or have its oxygen absorbing capacity. Also, other elements which can be used in elemental or partially oxidized form are sodium, manganese, iodine, sulfur, and phosphorous. These elements are also not as effective as iron because they do not have the oxygen absorbing capacity of iron, the rate of oxygen absorption of iron, or both. The oxygen absorbing salt may be sodium chloride or any other suitable food compatible salt including, but not-limited to, sodium sulfate, potassium chloride, ammonium chloride, ammonium sulfate, calcium chloride, sodium phosphate, calcium phosphate, and magnesium chloride.

A carrier resin for the oxygen absorbing material is preferably polyvinylchloride plastisol. Polyvinylchloride plastisol is a known resin for lining the inner surface of container caps. Other resins that may be used as the carrier resin for the oxygen absorbing material and can also serve as suitable sealants include, without limitation, high density polypropylene, high density polyethylene, acrylic, vinyl acetate ethylene copolymer, ethylene vinyl acetate, vinyl acetate homopolymer, acetate ethylene copolymer, plasticized vinyl chloride, oxidized polyethylene homopolymer, and polyurethane. When polyvinylchloride plastisol is used as the carrier resin, up to 75% by weight of liner 12 may be 200 mesh iron, a preferred oxygen absorbent.

Liner 12 is prepared by dispersing the oxygen absorbents within the carrier resin (in a viscous liquid state) by mixing in an electric, high-speed mixer. Liner 12 is then sprayed onto the inner surface of cap 11 in liquid form according to methods known in the art. Liner 12 adheres to cap 11. Cap 11 and liner 12 are then heated (to about 204.4°C (400°F) for 2 1/2 minutes) to solidify liner 12. Fig. 2 is a perspective view showing liner 12 coated on the inner surface of cap 11.

Cap 11 is attached to a container by first heating cap 11 until liner 12 softens. Cap 11 is then threaded onto the container, forming threads in liner 12 corresponding to grooves 13 in cylindrical portion 21 of cap 11. As shown in Fig. 3, cap 11 securely fits over the opening of container 15. Liner 12 seals cap 11 to container 15. Thus, liner 12 insures a tight fit between cap 11 and container 15 and facilitates the sealing function.

In addition, liner 12 absorbs oxygen within container 15 without the need for additional layers, such as cover layers or adhesive layers. The invention provides an economical and practical method for absorbing oxygen within a container by combining the adhesive function (affixing liner 12 to cap 11), the oxygen absorbing function, and the container sealing function in a single element: liner 12.

Fig. 4 is a side view of an alternative embodiment of the present invention. In the illustrated embodiment, cap 11 has a peripheral liner 30 disposed around the intersection of base portion 20 and cylindrical portion 21. Peripheral liner 30 extends over grooves 13 such that grooves will be formed in peripheral liner 30 as cap 11 is attached to a container. This ensures sealing cap 11 to the container. Peripheral liner 30 does not include an oxygen absorbent.

The embodiment illustrated in Fig. 4 also includes a central liner 31. Central liner 31 is disposed on the inner surface of base portion 20. Central liner 31 is centrally disposed and circular in the illustrated embodiment, but any shape or thickness may be used. Central liner 31 contains an oxygen absorbent that absorbs oxygen within the container to which cap 11 is attached. The oxygen absorbent is dispersed in central liner 31 as discussed above. Peripheral liner 30 and central liner 31 are both sprayed into cap 11 according to methods known in the art, and then heated to solidify.

Fig. 5 is a top view of the embodiment illustrated in Fig. 4. This embodiment conserves both the carrier resin material used for the liners and the oxygen absorbents.

The following examples are presented to illustrate the present invention; they are not intended to limit it.

### Example 1:

Polyvinylchloride plastisol in an amount of 10.35 grams was blended with 12.51 grams of 200 mesh iron containing 2% sodium chloride. The blending was done in an electric, high-speed mixer. A sample of the resulting liner material was coated on the inner surface of a container cap. The container cap was placed in a 500cc mason jar containing 100cc of oxygen. A one-eighth-inch hole was drilled in the lid of the mason jar with a septum placed over the hole to prevent oxygen from leaking out of the container. The container was left at room temperature at 100% relative humidity within the jar, and the amount of oxygen absorbed over time by the cap liner was measured. This procedure was repeated two times using different weights of liner material inside the cap. The results are tabulated below.

| **Oxygen Absorbed Over Time (cc)** | | | | |
|---|---|---|---|---|
| | Sample #1 | Sample #2 | Sample #3 | Average |
| Time | (1.47 g*) | (1,71 g*) | (1.51 g*) | (1.56 g*) |
| 22 hrs | 10 | 10 | 10 | 10 |
| 46 hrs | 15 | 14 | 15 | 15 |
| 96 hrs | 24 | 22 | 24 | 23 |
| 184 hrs | 37 | 32 | 34 | 34 |
| 234 hrs | 37 | 32 | 37 | 35 |
| 330 hrs | 51 | 41 | 48 | 47 |

| | | | | |
|---|---|---|---|---|
| * Weight of liner coated on inner surface of cap. | | | | |

### Example 2:

Polyvinyl chloride plastisol in an amount of 8.40 grams was blended with 5.17 grams of 200 mesh iron containing 2% sodium chloride in an electric, high-speed mixer. A sample of the resulting liner composition was coated on the inner surface of a container cap, which was placed in a 500cc mason jar containing 100cc of oxygen. A one-eighth-inch hole was drilled in the lid of the mason jar with a septum placed over the hole to prevent oxygen from leaking out of the container. The container was left at room temperature at 100% relative humidity within the jar, and the amount of oxygen absorbed by the liner over time was measured. The procedure was repeated two times using different weight samples of liner within the cap. The results are tabulated below.

| **Oxygen Absorbed Over Time (cc)** | | | | |
|---|---|---|---|---|
| | Sample #1 | Sample #2 | Sample #3 | Average |
| Time | (1.47 g*) | (1.71 g*) | (1.51 g*) | (1.56 g*) |
| 22 hrs | 8 | 8 | 8 | 8 |
| 46 hrs | 12 | 12 | 12 | 12 |
| 96 hrs | 26 | 19 | 21 | 22 |
| 184 hrs | 46 | 30 | 30 | 35 |
| 234 hrs | 52 | 33 | 30 | 38 |
| 330 hrs | 61 | 43 | 41 | 48 |

| | | | | |
|---|---|---|---|---|
| * Weight of liner coated on inner surface of cap. | | | | |

The results of both Examples 1 and 2 show good oxygen absorption using the present invention. Using the invention, the results are achieved with reduced material and fabrication time.

## Claims

1. A container cap (11) comprising:
a base portion (20) having a perimeter;
a substantially cylindrical portion (21) extending perpendicularly from said perimeter of said base portion and defining an inner surface of said container cap; and
a resin liner (12);
said resin liner being disposed in direct contact with said inner surface of said container cap and adhered to said inner surface with sufficient contact force to avoid additional mechanical sealing mechanism, said liner having an oxygen absorbent dispersed throughout; and
said container cap being adapted to seal an opening in a container (15) and to absorb oxygen within said container;
characterized in that:
said resin liner is entirely uncovered; and
said oxygen absorbent is selected from the group consisting of 200 mesh iron, aluminum, copper, zinc, titanium, magnesium, tin, sodium, manganese, iodine, sulphur, phosphorus, sodium chloride, sodium sulfate, potassium chloride, ammonium chloride, ammonium sulfate, calcium chloride, sodium phosphate, calcium phosphate, glucose oxidase, and magnesium chloride.

2. A container cap as claimed in claim 1 wherein said line (12) is polyvinylchloride plastisol.

3. A method for removing oxygen from a container (15) comprising:
attaching an oxygen absorbing liner (12) to a container cap (11); and
placing the cap over an opening in the container (15);
said liner being disposed in direct contact with said inner surface of said container cap and adhered to said inner surface with sufficient contact force to avoid additional mechanical sealing mechanisms, said liner having an oxygen absorbent dispersed throughout;
characterized in that:
said resin liner is entirely uncovered; and
said oxygen absorbent is selected from the group consisting of 200 mesh iron, aluminum, copper, zinc, titanium, magnesium, tin, sodium, manganese, iodine, sulphur, phosphorus, sodium chloride, sodium sulfate, potassium chloride, ammonium chloride, ammonium sulfate, calcium chloride, sodium phosphate, calcium phosphate, glucose oxidase, and magnesium chloride.

4. A method as claimed in claim 3 wherein the line (12) is polyvinylchloride plastisol.

5. A method as claimed in claim 3 wherein the line (12) is attached to the inner surface of the container cap (11) by spraying the liner in liquid form onto the inner surface.

## Patentansprüche

1. Behälterkappe (11), umfassend
einen Basisteil (20) mit einer äußeren Begrenzung,
einen im wesentlichen zylinderförmigen Teil (21), der sich senkrecht von der äußeren Begrenzung des Basisteils erstreckt und eine innere Oberfläche der Behälterkappe definiert, sowie
eine Harzauskleidung (12),
wobei die Harzauskleidung in direktem Kontakt mit der inneren Oberfläche der Behälterkappe angeordnet ist und mit ausreichendem Kontaktdruck haftend mit der inneren Oberfläche verbunden wird, um zusätzliche mechanische Dichtungsmechanismen zu vermeiden, wobei in der Auskleidung durchgehend ein Sauerstoffabsorptionsmittel dispergiert ist, und
die Behälterkappe so hergerichtet ist, dass sie eine Öffnung in einem Behälter (15) versiegelt und Sauerstoff innerhalb dieses Behälters absorbiert,
dadurch gekennzeichnet, dass die Harzauskleidung völlig unbedeckt ist und das Sauerstoffabsorptionsmittel aus der aus Eisen von 200 mesh, Aluminium, Kupfer, Zink, Titan, Magnesium, Zinn, Natrium, Mangan, Iod, Schwefel, Phosphor, Natriumchlorid, Natriumsulfat, Kaliumchlorid, Ammoniumchlorid, Ammoniumsulfat, Calciumchlorid, Natriumphosphat, Calciumphosphat, Glucoseoxidase und Magnesiumchlorid bestehenden Gruppe ausgewählt wird.

2. Behälterkappe nach Anspruch 11, in der die Auskleidung (22) ein Polyvinylchloridplastisol ist.

3. Verfahren zur Entfernung von Sauerstoff aus einem Behälter (15), umfassend
das Verbinden einer sauerstoffabsorbierenden Auskleidung (12) mit einer Behälterkappe (11) und
Aufbringen der Kappe auf eine Öffnung im Behälter (15),
wobei die Auskleidung in direktem Kontakt mit der inneren Oberfläche der Behälterkappe angeordnet ist und mit ausreichendem Kontaktdruck haftend mit der inneren Oberfläche verbunden wird, um zusätzliche mechanische Dichtungsmechanismen zu vermeiden, wobei in der Auskleidung durchgehend ein Sauerstoffabsorptionsmittel dispergiert ist,
dadurch gekennzeichnet, dass die Harzauskleidung völlig unbedeckt ist und das Sauerstoffabsorptionsmittel aus der aus Eisen von 200 mesh, Aluminium, Kupfer, Zink, Titan, Magnesium, Zinn, Natrium, Mangan, Iod, Schwefel, Phosphor, Natriumchlorid, Natriumsulfat, Kaliumchlorid, Ammoniumchlorid, Ammoniumsulfat, Calciumchlorid, Natriumphosphat, Calciumphosphat, Glucoseoxidase und Magnesiumchlorid bestehenden Gruppe ausgewählt wird.

4. Verfahren nach Anspruch 3, bei dem die Auskleidung (12) Polyvinylchloridplastisol ist.

5. Verfahren nach Anspruch 3, bei dem die Auskleidung (12) durch Aufsprühen der Auskleidung in flüssiger Form auf die innere Oberfläche mit der inneren Oberfläche der Behälterkappe (11) verbunden wird.

## Revendications

1. Bouchon de conteneur (11) comprenant :
une portion de base (20) ayant un périmètre ;
une portion sensiblement cylindrique (21) s'étendant perpendiculairement depuis ledit périmètre de ladite portion de base et définissant une surface intérieure dudit bouchon de conteneur ; et
une couche de résine (12) ;
ladite couche de résine étant disposée en contact direct avec ladite surface intérieure dudit bouchon de conteneur et adhérant à ladite surface intérieure avec une force de contact suffisante pour éviter l'usage d'un mécanisme d'étanchéité mécanique additionnel, ladite couche ayant un absorbant d'oxygène qui est dispersé dans toute sa masse ; et
ledit bouchon de conteneur étant adapté pour fermer de façon étanche une ouverture dans un conteneur (15) et pour absorber l'oxygène contenu dans ledit conteneur ;
caractérisé en ce que :
ladite couche de résine est entièrement découverte ; et
ledit absorbant d'oxygène est choisi dans le groupe consistant dans le fer à 200 mesh, l'aluminium, le cuivre, le zinc, le titane, le magnésium, l'étain, le sodium, le manganèse, l'iode, le soufre, le phosphore, le chlorure de sodium, le sulfate de sodium, le chlorure de potassium, le chlorure d'ammonium, le sulfate d'ammonium, le chlorure de calcium, le phosphate de sodium, le phosphate de calcium, l'oxydase de glucose et le chlorure de magnésium.

2. Bouchon de conteneur selon la revendication 1 dans lequel ladite couche (12) est en plastisol de chlorure de polyvinyle.

3. Procédé pour enlever l'oxygène dans un conteneur (15) comprenant :
fixer une couche (12) absorbant l'oxygène sur un bouchon de conteneur (11) ; et
placer le bouchon sur une ouverture du conteneur (15) ;
ladite couche étant disposée en contact direct avec ladite surface intérieure dudit bouchon de conteneur et adhérant à ladite surface intérieure avec une force de contact suffisante pour éviter l'utilisation de mécanismes de fermeture mécanique additionnels, ladite couche ayant un absorbant d'oxygène dispersé dans toute sa masse ;
caractérisé en ce que :
ladite couche de résine est entièrement découverte ; et
ledit absorbant d'oxygène est choisi dans le groupe consistant dans le fer à 200 mesh, l'aluminium, le cuivre, le zinc, le titane, le magnésium, l'étain, le sodium, le manganèse, l'iode, le soufre, le phosphore, le chlorure de sodium, le sulfate de sodium, le chlorure de potassium, le chlorure d'ammonium, le sulfate d'ammonium, le chlorure de calcium, le phosphate de sodium, le phosphate de calcium, l'oxydase de glucose, et le chlorure de magnésium.

4. Procédé selon la revendication 3, dans lequel la couche (12) est en plastisol de chlorure de polyvinyle.

5. Procédé selon la revendication 3 dans lequel la couche (12) est attachée à la surface intérieure du bouchon de conteneur (11) par pulvérisation de la couche sous forme liquide sur la surface intérieure.
